

April 7, 1936.

A. C. CLIFFORD

**2,036,256**

# FIBROUS ELECTRICAL INSULATION AND PREPARATION THEREOF

Filed Nov. 6, 1931

FIG. 1.



Fig. 2



INVENTOR  
A. C. CLIFFORD  
BY E. R. Nowlan  
ATTORNEY

## UNITED STATES PATENT OFFICE

2,036,256

FIBROUS ELECTRICAL INSULATION AND  
PREPARATION THEREOFAlbert C. Clifford, Elizabeth, N. J., assignor to  
Western Electric Company, Incorporated, New  
York, N. Y., a corporation of New York

Application November 6, 1931, Serial No. 573,347

17 Claims.

(Cl. 28—58)

This invention relates to the preparation of fibrous materials, and more particularly to a method of purifying fibrous materials such as cotton for use as insulation on electrical conductors.

5 Objects of the invention are to remove substantially all foreign materials from and to purify fibrous materials such as cotton in fibrous, stranded or textile form by improved methods that are more convenient, economical and efficient than methods heretofore known or used.

Briefly, one embodiment of the invention contemplates enclosing the material in a pressure chamber and circulating a bleaching solution therethrough, whereby a very substantial portion 15 of the natural oils and waxes contained in the material are removed. The solution is then drained from the chamber, and clear rinse water may or may not be circulated through the material, as desired. In order to effect further purification, a saturated solution of calcined gypsum is circulated through the material, after which it 20 may again be rinsed with clear water. Removal of the material from the pressure chamber, and thorough drying completes the process.

25 Other features and advantages of the invention will become apparent from the following detailed description of one embodiment thereof, by means of which the method may be practiced, reference being had to the accompanying drawings wherein

30 Fig. 1 is an elevational view partly broken away of a material treating apparatus, and

Fig. 2 is a plan view thereof.

Referring now to the drawing in which like 35 numerals designate like parts throughout the several views, the numeral 10 designates a cylindrical vessel having a removable cover 11 which may be securely fastened in pressure-tight relation to the vessel 10 by means of a plurality of latches 12.

40 The vessel 10 is provided with a bottom 13, and partitions 14 and 15, which act as false bottoms and divide the interior of the vessel into a plurality of chambers 17, 18 and 19. The partition 14 which may or may not be employed as 45 desired is provided with a plurality of openings 21 which permit the flow of liquid from the chamber 17 into the chamber 18, and the partition 15 is provided with a large central opening 22, which leads into a pipe 23, extending through the chamber 19 and through the bottom of the vessel 10 where it connects with a pipe 25. The partition 15 is provided with a plurality of openings 26—28, which are in alignment with corresponding openings in the partition 14 through which openings 50 hollow perforated spindles 27 protrude, so as

to permit the flow of a fluid to and from chambers 17 and 19 without the fluid flowing into chamber 18.

In practice the cotton strands which are to be purified are wound or reeled somewhat loosely 5 on porous flexible hollow cylindrical cores or bobbins 29, which are longitudinally compressible. A plurality of the packages of cotton thus formed are placed on the perforated spindles 27, within the vessel 10, as shown at 30. The packages 30 10 are placed one above the other on each spindle, until each pile of packages extends above its associated spindle. A pressure plate 32 which covers the top of the uppermost package, and which is provided with a stem 36 which may enter 15 the upper end of the perforated tube, is then placed over each of the piles of packages. The cover 11 is provided on the inside thereof with a plurality of spring pressed plungers 31 so spaced and aligned that one plunger shall be directly 20 above each of the spindles 27 when the cover 11 is placed in position. As the cover is lowered into position, each of the plungers 31 compresses one of the piles of packages of cotton 30, until the tops of the piles are substantially flush with 25 the upper ends of the spindles and the bottoms of the piles are urged against the supporting members 34 on the partition 14. The plungers are provided with head portions 33 which are urged against the pressure plates. It is thus ap- 30 parent that the plungers 31 will exert a pressure on plate 32, which will be transmitted to the packages of cotton, and that since the bottom of each pile is pressed against the supporting member 34, and the upper end of the pile is 35 covered by the pressure plate, any fluid that flows up into the spindles 27 and out through the perforations to the interior of the cylindrical aperture through the piles, is prevented from flowing out of the ends of the cylindrical aperture, and 40 under pressure it will flow transversely through the packages of cotton, and out into the chamber 17.

The bottom 13 of the vessel 10 has an opening 45 33 therein, at which point a pipe 35 is connected 45 so as to convey fluid to and from the chamber 19. The pipes 25 and 35 lead from the chambers 18 and 19 respectively, in the vessel 10, to a reversing valve 37, from which pipes 38 and 39 lead to the inlet and outlet parts respectively 50 of a centrifugal pump 41 driven by an electric motor 42. An expansion tank 43 is positioned above the pump 41 and a drain pipe 45 leads from the bottom of the tank 43 to the pipe 38 so as to discharge the contents of the expansion 55

tank into the centrifugal pump 41. The expansion tank 43 is also provided with an overflow pipe 46 leading to a waste discharge system of any suitable type (not shown), to prevent the contents of the expansion tank from overflowing.

Steam inlet pipes 48 and 49 are provided below the vessel 10 to permit the introduction of steam into the pipes 25 and 35 respectively, and the vessel 10 is provided with pressure gauges 51 and 52 which indicate the pressures within the chambers 17 and 19 respectively. The vessel 10 is also provided with an overflow pipe 53 leading into the expansion tank 43, in which pipe is positioned a thermometer 55, by means of which the temperature within the chamber 17 may be ascertained, and a valve 56 is provided to regulate the flow of fluid through the pipe 53 when desired. A drain valve 57 is provided adjacent to and in the same line with the reversing valve 37, to drain the fluid from the system into a waste discharge pipe 59 which leads to a waste discharge system (not shown). An auxiliary drain pipe 60 leads from the pipe 25 through a valve 61 to the waste discharge pipe 59. A water supply pipe 63 is connected from a source of water (not shown) through a valve 64 to the expansion tank 43.

When a quantity of cotton has been made up into packages 30, and the cotton is to be purified, the packages are disposed on the spindles 27 until they are filled, as previously described. The cover 11 is then lowered into place, and is securely latched, and the purifying solution is admitted into the expansion tank 43. The pump is then started, with the reversing valve 37 preferably adjusted so that the purifying fluid flows from the valve, through the pipe 35, through the aperture 33, into the chamber 19, up through the spindles 27, out through the perforations in the spindles and through the cotton into the chamber 17, down to and through the pipe 23, out through the pipe 25, back to the valve 37, and back to the pump. It is continuously circulated by the pump through the same path. This is commonly designated as circulation from inside to outside.

It may become desirable to circulate the purifying fluid in the opposite direction. The path of flow will then be from the valve 37, through the pipes 25 and 23, up into the chamber 17, through the cotton and through the perforations in the hollow spindles, down through the spindles, out through the aperture 33, and through the pipe 35 to the reversing valve, and then to the pump. This is commonly designated as circulation from outside to inside.

It frequently is desirable to permit a portion of the purifying fluid in the apparatus to be drawn off during the purifying process. For this purpose, the auxiliary drain pipe 60 has been provided. The valve 61 may be adjusted so that any desired quantity per time interval, of purifying fluid, may drain off and flow to the waste discharge system. This will permit a substantially equal quantity of fresh purifying fluid to enter the apparatus from the expansion tank 43. By means of this arrangement, purifying fluid that is contaminated with impurities is continually escaping from the apparatus, and the concentration of impurities is kept low.

While the above described apparatus, which is commonly known as a "Franklin dyeing machine", is well suited for performing the process which will hereinafter be described in detail,

other forms of apparatus, such for example as the "Thies dyeing machine" and the "Obermaier dyeing machine", which operate on a similar principle, may be satisfactorily employed. Also, since the above described apparatus may be employed in numerous ways in preparing and treating fibrous materials, in order that the invention may be clearly understood, the preferred embodiment, by means of which the method may be practiced, will now be described.

In general, the impurities that may be found in cotton are the non-ionizable impurities, among which may be included the natural oils and waxes, and the ionizable or electrolytic impurities, which consist principally of inorganic compounds, such as compounds containing the alkali metals. The non-ionizable impurities may not, under certain circumstances, have a deleterious effect upon the electrical characteristics of the cotton. It may sometimes be advantageous, however, in the preparation of cotton for use as insulating material, to remove the natural oils and waxes, as the cotton is thereby softened, which may result in easier handling and processing during subsequent operations. For some uses other than as electrical insulation, it is sometimes very desirable to remove the natural oils and waxes, deleterious effects being observable in the final product if these impurities are permitted to remain in the cotton.

The removal of the ionizable impurities is very important when cotton is to be used for insulating purposes. These impurities, if permitted to remain in the cotton, may, under the influence of moisture, become rather highly conductive, thus greatly reducing the insulation resistance of the cotton, thereby partially destroying its value as a dielectric material.

The removal of both types of impurities may be accomplished in the above described apparatus, without disturbing or removing the contents of the machine during the process. It has been found preferable to perform the operation of removing non-ionizable impurities before removing the ionizable impurities, for the reason that the reagent by means of which the oils and waxes are removed may form and leave in the cotton, substances which would have a deleterious effect upon the electrical characteristics of the cotton.

The cotton preferably spun into strands, is wound upon the porous flexible cores, thus forming the packages hereinbefore described. The packages are placed on the spindles in the container 10, also in the manner also hereinbefore described, and the cover 11 is secured in place.

The liquid that has been found particularly suited to remove the natural oils and waxes from the cotton is a water solution of sodium hydroxide, having a concentration of approximately one pound of the hydroxide per one hundred gallons as water. Instead of sodium hydroxide, other suitable reagents may be employed, such for example as peroxides, and other hydroxides. The solution may be prepared in any convenient container, and then introduced into the expansion tank, or it may be prepared in the expansion tank, by admitting water from the source of supply, adding the sodium hydroxide, and stirring to effect complete solution of the base. The system is then ready for circulation of the solution, which may be accomplished by adjusting the reversing valve to permit the solution to enter the chamber 10, after which the pump is started. It has been found preferable to circulate the solution from

inside to outside initially, a path that has been previously described. However, it is not essential that the solution be circulated in this path, and satisfactory results may be obtained by initially 5 circulating the solution from outside to inside.

Also, as many reversals of direction of flow may be effected during the process as may seem desirable. The most satisfactory results may be obtained by keeping the solution heated during 10 the process, and this may be accomplished by admitting steam through the steam inlet pipes provided for that purpose. It is advisable to permit the temperature to rise not higher than 130° Fahrenheit, as the sodium hydroxide may sometimes have a corrosive or disintegrating action at temperatures higher than the above. Also, it has been found that the best results are obtained by maintaining the temperature about 90° Fahrenheit.

20 After the solution has been circulated a predetermined length of time, the pump may be stopped, and the solution, containing the oils and waxes have been removed, may be drawn off through the outlet and permitted to escape to the drain. The circulation of the sodium hydroxide may have left in the cotton fibres small quantities of water soluble impurities, such as the base itself or compounds derived therefrom. Portions of these impurities may conveniently be removed, 25 before the further purification of the cotton with reagents, by circulating clear water through the cotton, and the amount of impurities to be subsequently removed will thereby be reduced. The washing may be done by introducing clear water 30 into the expansion tank, starting the pump and circulating the water for a short period of time, after which it is permitted to escape through the drain. It should be understood that the rinsing with clear water is not a required operation, and 35 that it may be performed or not, as desired.

The purifying liquid that is employed to remove the ionizable impurities consists of a saturated solution of best grade calcined gypsum in water. One form of calcined gypsum, which is also known 40 as plaster of Paris, is obtainable commercially as No. 1 moulding plaster. The operations of dissolving the calcined gypsum and of circulating the solution may be performed in a manner similar to those employed in preparing and circulating the sodium hydroxide solution. In connection with the circulation of this purifying solution it has been found preferable to circulate initially from inside to outside of the packages 45 of cotton, but the initial circulation may be in the opposite direction, and the direction of circulation may be changed as many times as desired during the process.

It has been found that the purification may be satisfactorily conducted at temperatures ranging 50 from 90° to 100° Fahrenheit. Between these temperature limits gypsum exhibits substantially maximum solubility. While particularly satisfactory purification of cotton may be accomplished between these temperature limits, it is to be understood 55 that the process may satisfactorily be conducted at lower or higher temperatures, if such variation is found to be desirable.

After the process has been conducted a predetermined length of time, the pump may be 60 stopped, and the contaminated solution may be permitted to escape from the apparatus to the waste discharge system. The packages of cotton may then be removed from the vessel 65, or if it may appear desirable to give the cotton a rinse, clear water may be introduced into the expansion

tank, and may be circulated for a few minutes in the same manner in which the purifying solution was circulated. The cotton may then be removed from the apparatus and thoroughly dried in any convenient manner.

5 The use of calcined gypsum affords numerous advantages which make the process of purifying cotton described herein particularly desirable. The gypsum is carried into the fibres of the cotton to a large extent and in a very satisfactory 10 manner. Furthermore, calcined gypsum is an inexpensive material, and the cost of preparing the cotton for use as insulation is quite low.

15 While the exact function performed by the calcined gypsum in the above described method of treating cotton is not clearly understood, it is believed that entire molecules or parts of molecules of the readily soluble and ionizable inorganic impurities found in or on the fibres of cotton are replaced by molecules or parts of molecules of the 20 relatively insoluble and non-ionizable calcium sulphate in the solution of calcined gypsum employed in treating the cotton. Experiments seem to indicate that the cotton fibres have an affinity for the calcium cations present in the solution of calcined gypsum and that the calcium cations are 25 substantially irreversibly adsorbed by the cotton fibres in preference to the more readily ionizable cations present in the cotton, such, for example, as those of the alkali metals. Whatever the true 30 function of the solution of calcined gypsum may be, the use of such a solution for treating cotton in accordance with the method hereinbefore described results in such a marked improvement in 35 the electrical insulating properties of the cotton that it may be satisfactorily substituted for the usual insulating silk in many cases, particularly for use under conditions of high humidity where the presence of ionizable impurities is deleterious.

40 Although the preferred path of circulation has been found to be from inside to outside of the packages of cotton, the invention is not limited to that method of operation, as satisfactory results can be obtained by circulating the solution from outside to inside of the packages. Similarly, 45 both methods may be used alternately during the process of purifying the cotton, and there may be as many reversals of the direction of flow as may seem desirable.

50 While the method of treating cotton has been described herein as a single process, consisting of steps wherein two widely different types of impurities may be removed from cotton, it is not intended that the process shall be limited to these steps. Depending upon the uses to which the 55 cotton may be applied, it is intended to be within the scope of this invention, that the purification of cotton may be confined exclusively to the process for removing natural oils and waxes, or 60 that it may be confined to the removal of ionizable impurities.

65 It should be understood that while the process of purifying cotton herein described is well adapted for the purification of cotton in the form of strands wound into packages, it is not confined to this arrangement alone, as the process is well suited to the purification of cotton in all forms such, for example, as unspun raw cotton fibre or 70 woven cotton fabric.

75 Although the description of the invention has included but a single method whereby it may be practiced, the invention is not to be construed as limited to that method, as many modifications in the method and apparatus may be made, within the scope of the appended claims.

What is claimed is:

1. The method of treating strands of cotton to improve their insulating properties which comprises washing said strands with a solution of calcined gypsum.
2. The method of treating cotton textiles to improve their insulating characteristics which comprises treating the textiles with a solution of calcined gypsum under pressure.
10. The method of treating cotton strands to improve their insulating characteristics which comprises placing the strands in a pressure chamber, circulating a saturated solution of calcined gypsum around the strands, removing the gypsum solution, and circulating clear water around the strands.
15. The method of treating cotton strands to improve their insulating characteristics which comprises winding the strands on porous bobbins, placing the windings in a pressure chamber, circulating a solution of calcined gypsum around the windings under pressure, removing the gypsum solution, circulating clear water around the windings, removing the water, and drying the windings.
20. The method of removing impurities from cotton materials to improve their insulating properties which comprises treating the materials with a solution of sodium hydroxide, and treating the material with a solution of calcined gypsum.
25. The method of removing non-ionizable and ionizable impurities from cotton, which comprises placing the cotton in a container, circulating a solution of sodium hydroxide through the cotton under pressure, and circulating a saturated solution of calcined gypsum through the cotton.
30. The method of preparing insulating material, which comprises removing the ionizable materials from cotton by repeatedly forcing a hot solution of calcined gypsum under pressure through a mass of the cotton.
35. The method of preparing insulating material, which consists in forcing a saturated solution of calcined gypsum under pressure at a temperature of from 90° to 100° Fahrenheit through a mass of cotton and thereby removing the ionizable impurities from the cotton.
40. The method of removing ionizable impurities in cotton, which consists in forcing a solution of calcined gypsum under pressure at a temperature of from 90° to 100° Fahrenheit through a mass of cotton in one direction, and then forcing a like solution through the mass of cotton in another direction.
45. The method of preparing insulating material, which consists in forcing a hot alkaline solution under pressure through a mass of cotton, and then forcing a hot solution of calcined gypsum under pressure through the cotton.
50. The method of preparing insulating material, which consists in forcing a solution of sodium hydroxide under pressure at a temperature not exceeding 130° Fahrenheit through a mass of cotton, washing the cotton with water, then forcing a saturated solution of calcined gypsum under pressure at a temperature of from 90° to 100° Fahrenheit through the cotton, and washing the cotton with water.
55. The method of preparing insulating material which comprises replacing the ionizable impurities in cotton by treating the cotton with a solution of calcined gypsum.
60. An insulating material comprising cotton fibres characterized by being substantially free from non-ionizable and ionizable impurities and by having thereon calcium bearing material irreversibly adsorbed thereby from a saturated solution of calcined gypsum.
65. The method of preparing insulating material, which comprises removing natural oils and waxes from cotton, and then treating the cotton with a solution of calcined gypsum to remove ionizable impurities therefrom.
70. The method of preparing insulating material, which comprises treating a mass of cotton with a solution of a reagent falling within the empirical class of hydroxides and peroxides, and then treating the cotton with a solution of calcined gypsum to remove ionizable impurities therefrom.
75. As a new article of manufacture, electrical insulating material comprising spun cotton which has been freed from the major portion of its natural oils and waxes and from all non-ionizable and all ionizable impurities and having thereon an irreversibly adsorbed calcium bearing material absorbed thereby from a solution of calcined gypsum.
80. An insulating material comprising spun cotton which has substantially constant electrical characteristics under varying conditions of humidity and which has been freed from substantially all of its natural oils and waxes and all impurities and having thereon an irreversibly adsorbed calcium bearing material absorbed thereby from a solution of calcined gypsum.

ALBERT C. CLIFFORD.